

Nov. 9, 1937.

W. B. TUCKER

2,098,603

COT

Filed Feb. 7, 1935

*Fig. 1*



*Fig. 4*



*Fig. 2*



*Fig. 5*



*Fig. 3*



Inventor  
William B. Tucker  
by  
Walter + Langman

Attorney

## UNITED STATES PATENT OFFICE

2,098,603

## COT

William B. Tucker, Lancaster, Pa., assignor to  
 Armstrong Cork Company, Lancaster, Pa., a  
 corporation of Pennsylvania

Application February 7, 1935, Serial No. 5,378

10 Claims. (Cl. 19—143)

My invention relates to cots and more particularly to covers in the form of preformed cork composition cots adapted to be applied to rolls or other surfaces to be covered, and preferably held 5 in position by means of adhesive, although my invention is also applicable to cots intended to be held in place solely by friction.

Cork composition cots have been used with considerable success in the spinning and drawing of 10 cotton fibers. They are also used as coverings for typewriter feed rolls, pulleys and the like. In many such uses, it is desirable to have a relatively soft working surface, and, consequently, the cots are more or less compressible along a direction 15 parallel to their axes.

Cots are generally secured to the rolls or other surfaces which they cover by means of adhesive, although in some instances they are held in position solely by friction. It is customary to form 20 the cots with an inner diameter slightly less than the outer diameter of the roll to which it is to be applied, say  $\frac{1}{64}$ " less for the usual spinning cots, and force the roll into the cot, thus placing the cot under pressure along a direction parallel to its axis. The frictional engagement of the cot 25 with the roll exerts considerable force on the cot, and, as a result, the cot is compressed to a considerable extent and does not properly cover the roll to which it is applied. The compression of 30 the cork composition also results in a denser working surface which may, in some instances, be objectionable.

It is an object of my invention to provide a cot in which the density of the body, which may be 35 cork composition, may be relatively low and the compressibility of the composition, consequently, relatively high, which cot is, nevertheless, relatively rigid along a direction parallel to its axis. In my preferred embodiment, longitudinal compression is inhibited by means of a tenent coating applied to at least a portion of a surface of the cot lying along a line parallel to the axis of the cot.

A further object of my invention is to provide a 45 cot having a tenent coating applied to a surface thereof of which coating may be rendered adhesive and serve to secure the cot to a roll or other surface it is to cover.

In order that my invention may be more readily 50 understood, I will describe the same in conjunction with the attached drawing, in which—

Figure 1 is a side elevation of a cotton spinning roll having two cots applied thereto, illustrating the effect of compression of a cot incident to application to a roll;

Figure 2 is an oblique view of a cot embodying my invention;

Figure 3 is a diagrammatic view of a mechanism commonly employed for applying cots to rolls; and

Figures 4, 5, 6 and 7 are sectional views illustrating modifications of my invention.

Figure 1 shows, diagrammatically, a cotton spinning roll 2 having arbors 3 and 4 covered with cots 5 and 6 respectively. The cot 6 is of the usual type whereas the cot 5 embodies my invention. The chain lines 5' and 6' represent the size of the cots prior to application. It will be noted that they are identical in size prior to application, but that the applied cot 6 is compressed to about three-fourths the size of the cot 5. This compression may be due to a number of combining conditions. In the first place, the rolls are usually provided with a roughened surface 7 which serves to hold adhesive when the cots are adhesively secured and also serves to aid in frictionally holding the cots if they be applied without adhesive. The cots are generally made with an inner diameter slightly less than the outer diameter of the arbor as pointed out above, and in some instances the arbors will not be accurately machined. It is not uncommon to find arbors .008" to .010" oversize. This naturally increases the friction developed in the application of cots thereto.

In Figure 3, a cot assembly mechanism commonly employed in the art is shown with a cotton spinning roll in position with one cot applied to an arbor thereof and a second cot in the process of being assembled with the roll. 35 The mechanism includes a base 8 in which is mounted a spring urged hollow spindle 9 and a pressure applying rod 10 mounted in guideways 11 and 12. The rod 10 is movable toward the spindle 9 and is provided with an operating lever 13 secured to a quadrant 14, connected by a belt or chain 15 to a collar 16 secured to the rod 10; rotation of the quadrant in a counter-clockwise direction moving the rod 10 toward the spindle 9. In the application of cots to arbors, an entering 45 thimble 17 is placed over the end of a roll 18 and the opposite end of the thimble is entered into the spindle 9. A cot 19 is placed over the spindle 9, the spindle being of substantially lesser diameter than the inner diameter of the cot. The end 50 of the roll opposite to the end upon which the cot is to be applied is held in a suitable jaw 20 in the pressure applying rod 10. The quadrant 14 is now rotated in a counter-clockwise direction and the thimble 17 is urged into the cot, enter- 55

ing the roughened arbor surface 21 of the roll 18 into the cot 19, the spindle 9 retreating into the guide 22 upon compression of the spindle returning spring. Since the cots are of a compressible nature, particularly in a direction parallel to the axis thereof, they will be compressed to some extent by this assembly operation and, as a result, will not cover the entire arbor. As pointed out above, this compression is partly due to frictional engagement of the cot with the arbor and this frictional engagement is materially increased by the roughened surface 21.

A cot embodying my invention is illustrated in Figure 2. The cot shown is formed of a body of cork composition 23 having a renitent coating 24 applied to its inner wall. The coating 24 preferably extends over the entire inner surface of and in direct contact with the body, but it may be applied to any portion of the body so long as it serves to rigidify the body along a direction parallel to its axis or in the direction of pressure developed during assembly. The coating is preferably relatively thin, say .003", when dry, and should form a relatively stiff, unyielding film upon drying or setting. Any coating which serves this purpose will be satisfactory.

I have obtained good results using a .003" coating of water soluble adhesive such as hide glue. A coating of this type is desirable in that it may be utilized to secure the cot to the arbor, the assembly operation being performed by dipping the roll in water and then thrusting it rapidly into the cot. The roll is preferably positioned in the cot prior to any material weakening of the renitent coating by contact with the water on the roll.

In some instances it may be found desirable to provide a coating which will not be materially affected by moisture. While the use of a water soluble adhesive as the renitent coating will be found advantageous in certain instances, it is not essential that the renitent coating serve this purpose. For example, a suitable renitent coating might take the form of a resin dissolved in an appropriate solvent or applied in heated condition. A coating of lacquer will also serve this purpose. The renitent coating may be covered with an adhesive coating as shown in Figure 4.

A body of cork composition 25 has a renitent coating 26, say a resin or lacquer coating, and an adhesive coating 27. In this type of cot, the adhesive may or may not form a renitent coating, since compression along a direction parallel to the axis of the body 25 is limited by the coating 26.

It should be borne in mind while viewing the drawing that the thickness of the coatings is shown to an exaggerated scale for sake of clarity. The thickness of the coating will depend to some extent upon its renitent properties and also upon the density and compressibility of the untreated cot.

When a relatively low density material is employed, it may be found desirable to apply a renitent coating to the outer surface of the cot as well as to the inner surface. In Figure 5, a cork composition cot 28 is shown having a renitent coating 29 applied to the outer surface and a coating 30 applied to the inner surface. The outer coating is preferably one that may be readily removed by grinding, such as a film of nitro-cellulose lacquer and the inner coating may be a water soluble adhesive for example. The use of an outer coating entails, of course, the prob-

lem of removing the applied coating for it is desirable to have the cork composition exposed at the working surface. Cots are generally buffed after application to the roll in order to provide a true, smooth surface, and it is a simple matter to grind the renitent coating during this buffing operation.

In Figure 6 a cot is shown in which the renitent coating is applied in the form of helical strips 31, 32 and 33 extending along the inner surface 10 of the cot 34 and bonded directly thereto. The strips preferably extend from edge to edge in order to prevent compression and, while they are illustrated as helical strips, they could run parallel to the axis with equally satisfactory results. Any formation of coating may be used provided it serve to inhibit material longitudinal compression of the cots upon the application to rolls or other surfaces to be covered.

Figure 7 illustrates a further modification of my invention in which the renitent coating is applied only to the outer surface of the cot. The cork composition body is shown at 35 and the coating at 36. As illustrated, the coating may cover the entire outer surface or may be otherwise disposed. The coating 36, as in the embodiment of Figure 5, should be one that may be readily removed by grinding. This type of cot is particularly desirable for use in those places where the cot is held solely by friction. It is obvious, however, that an adhesive may be applied to the inner surface of the cot prior to application and the renitent coating 36 relied upon to prevent material compression along a direction parallel to the axis of the cot.

My invention is obviously of great advantage where relatively soft cork composition coverings are required, say 25 pounds or less in density. In the cotton spinning industry, for example, cots having a relatively soft cork composition working surface are generally employed. Since the resistance of the composition to compression along a direction parallel to the axis of the cot decreases in proportion to the increase in softness of the cork composition and decrease in density, the problem of assembly has become more prominent with the trend toward softer cork composition cots. By my invention the major problem is overcome, and rapid assembly, without material compression and consequent increase in density and hardness of the surface, is obviated.

In the embodiments of my invention shown in the drawing, the body of the cot is composed of cork composition. My invention is applicable to cots having bodies of other material of a compressible character, such for example as rubber bound compositions commonly used for type-writer feed rolls.

In order to determine the renitent qualities of a water soluble gelatine coating applied to the entire inner surface of cork composition cots, a number of samples were obtained from a single batch and some were coated on their inner surface with a layer of hide glue which was approximately .003" thick upon drying. The samples were all of substantially the same density, hole size, length and outside diameter. It was found that, upon the application of 15 pounds pressure along a direction parallel to the axis of the cots for one minute, the uncoated cots compressed about three times as much as those having the renitent coating applied thereto. For example, cots 1 1/8" long having an outer diameter of 1 3/2" and a hole size of 1 1/8" and a density of 27 pounds per cubic foot compressed .157" upon the appli-

cation of 15 pounds pressure, whereas similar cots embodying the renitent coating compressed but .060" upon the application of 15 pounds pressure.

- 5 It is intended by the statement, as used in the claims, that the entire body of the cot is readily compressible axially, to express the fact that the cot, without a renitent coating or coatings, would normally be readily compressible axially, and to thereby distinguish the cots of my invention from those cots which are inherently resistant to axial compression—such as fiber interlined cots or multi-ply structures possessing such characteristics.
- 10 15 While my invention has been described particularly in connection with cork composition cots for textile rolls, it will be understood that my invention is applicable to cots for other uses. It is, of course, particularly desirable where the 20 density of the composition is relatively low, but is, nevertheless, applicable to the more dense compositions commonly employed in industry.

While I have described and illustrated the preferred embodiment of my invention, it will be understood that the invention is not so limited but may be otherwise embodied with the scope of the following claims:

I claim:

1. A cot for covering rolls or the like, the entire body of which is readily compressible axially, comprising a hollow cylindrical body having a resilient working surface and a relatively thin, dried, renitent coating, capable of being rendered adhesive by the application of water thereto, applied directly to substantially the entire exposed inner surface of the body and rendering said cot resistant to axial compression upon application of the cot to a roll.
2. A cot for covering rolls or the like, the entire body of which is formed of cork composition and is readily compressible axially, comprising a hollow, cylindrical cork composition body having a resilient cork composition working surface and a dried renitent coating of gelatine glue, capable of being rendered adhesive by the application of water thereto, applied to substantially the entire exposed inner surface of the cork composition body and bonded thereto and rendering said cot resistant to axial compression upon application of the cot to a roll.
3. A cot for covering rolls or the like, the entire body of which is readily compressible axially, comprising a hollow cylindrical body of cork composition having a density of twenty-five pounds or less

per cubic foot and presenting a soft, resilient cork composition working surface, and a dried, renitent coating applied to the inner surface of the cork composition body and rendering said cot resistant to axial compression upon application of the cot 5 to a roll, said renitent coating constituting the sole means auxiliary to the body to render said cot resistant to axial compression upon application of the cot to a roll.

4. A cot for covering rolls or the like, the entire body of which is readily compressible axially, comprising a hollow, cylindrical body of cork composition having a density of twenty-five pounds or less per cubic foot, having a resilient 10 cork composition working surface and a relatively thin, dried renitent coating of gelatine glue, capable of being rendered adhesive by the application of water thereto, applied directly to substantially the entire exposed inner surface of the cork composition body and bonded thereto, said 15 renitent coating constituting the sole means auxiliary to the body to render said cot resistant to axial compression upon application of the cot to a roll.

5. A cot for covering rolls or the like, the entire body of said cot being formed of material of such character that it is compressible axially to an objectionable extent when subjected to frictional forces set up in applying the cot to a roll, comprising a hollow cylindrical body, having a resilient working surface and a dried, renitent coating applied to the body and rendering said cot resistant to such axial compression upon its application to a roll.

6. A cot in accordance with claim 5 in which the renitent coating is applied to the inner surface of the body and is capable of being rendered adhesive.

7. A cot in accordance with claim 5 in which the renitent coating is applied to substantially 40 the entire exposed inner surface of the body.

8. A cot in accordance with claim 5 in which the entire body is formed of cork composition and in which the renitent coating is applied to substantially the entire exposed inner surface thereof.

9. A cot in accordance with claim 5 in which the renitent coating is applied to the inner surface of the body and in which a dried coating of adhesive is disposed over a portion at least of the renitent coating.

10. A cot in accordance with claim 5 in which the renitent coating is applied to the outer surface of the body.

WILLIAM B. TUCKER.